# EUROPEAN PATENT SPECIFICATION

(11) **EP 0 588 342 B1**
(45) Date of publication and mention of the grant of the patent: **12.07.2000**
(21) Application number: 93114924.9
(22) Date of filing: 16.09.1993
(51) Int. Cl.: C21D 8/12, C22C 38/02

(54) **Grain-oriented electrical steel sheet and material having very high magnetic flux density and method of manufacturing same**
Kornorientierte Elektrobleche und Material mit sehr hoher magnetischer Flussdichte und Verfahren zur Herstellung dieser
Tôle d'acier électrique à grains orientés et matériau à haute densité de flux magnétique et procédé pour leur fabrication

(30) Priority: 17.09.1992 JP 24819492; 23.10.1992 JP 28648692
(43) Date of publication of application: 23.03.1994
(73) Proprietor: NIPPON STEEL CORPORATION, Tokyo 100 (JP)
(72) Inventor: Takashima, Kunihide, c/o Nippon Steel Corporation, Futtsu-shi, Chiba (JP); Kawamata, Ryutarou, c/o Nippon Steel Corporation, Futtsu-shi, Chiba (JP); Nakamura, Yoshio, c/o Nippon Steel Corporation, Futtsu-shi, Chiba (JP); Iwanaga, Isao, c/o Nippon Steel Corporation, Kitakyushu-shi, Fukuoka (JP); Abe, Norito, c/o Nippon Steel Corporation, Himeji-shi, Hyogo (JP)
(74) Representative: VOSSIUS & PARTNER

(56) References cited:
- EP-A- 0 101 321
- EP-A- 0 315 948
- EP-A- 0 339 475
- EP-A- 0 390 140
- EP-A- 0 390 142
- US-A- 4 642 141
- PATENT ABSTRACTS OF JAPAN, unexamined application, C field, vol. 15, no. 231, June 12, 1991 THE PATENT OFFICE JAPANESE GOVERNMENT page 45 C 840
- PATENT ABSTRACTS OF JAPAN, unexamined applications, C field, vol. 15, no. 7, January 09, 1991 THE PATENT OFFICE JAPANESE GOVERNMENT page 116 C 794
- PATENT ABSTRACTS OF JAPAN, unexamined applications, C field, vol. 12, no. 11, January 13, 1988 THE PATENT OFFICE JAPANESE GOVERNMENT page 120 C 468
- CHEMICAL ABSTRACTS, vol. 105, no. 2, July 14, 1986, Columbus, Ohio, USA IGUCHI, MASAO et al. "Direc- tional silicon steel strip with excellent magnetic pro- perties" page 237, column 2, abstract- -no. 10 195t
- CHEMICAL ABSTRACTS, vol. 117, no. 6, August 10, 1992, Columbus, Ohio, USA YOSHITOMI, YASUNARI et al. "Manufacture of anisotropic electromagnetic steel sheets having improved magnetic pro- perties" page 297, column 1, abstract- -no. 53 362k
- CHEMICAL ABSTRACTS, vol. 105, no. 2, July 14, 1986, Columbus, Ohio, USA IGUCHI, MASAO et al. "Directional silicon steel strip with excellent magnetic properties" page 2377, column 2, abstract-no. 10 194s

## Description

This invention relates to grain-oriented electrical steel sheet and material having very high magnetic flux density for use in the cores of transformers and the like in which {110} [001] Goss texture orientation is promoted to a high level, and a method of manufacturing same.

As a soft magnetic material, grain-oriented electrical steel sheet is used primarily for the core material of transformers and other electrical devices, and with respect to magnetic properties therefore has to have good excitation and core loss characteristics. Usually a B₈ (magnetic flux density at a magnetic field strength of 800 A/m) value is used to express excitation characteristics numerically and core loss characteristics are expressed as a W_{17/50} (core loss per kilogram of material that has been magnetized to 1.7 tesla at 50 Hz) value.

In recent years there has been a sharp increase in societal demands for energy saving and resource conservation, which has brought increased demands for lower core loss values and improved excitation properties in grain-oriented electrical steel sheet, with the demand for lower core loss properties being particularly strong.

Core loss consists of hysteresis loss and eddy current loss. Hysteresis loss depends on such factors as crystal orientation of the steel sheet (in other words, magnetic flux density), purity and internal stress, while factors such as electrical resistance, sheet thickness, grain size, magnetic domain size and steel sheet coating tension contribute to the eddy current loss.

After a long history of careful consideration in terms of production technology the limit has been more or less reached with respect to purity and internal stresses and the like. The silicon content of steel sheet has been raised in an attempt to increase electrical resistance and reduce eddy current loss, but a limit has been reached inasmuch as raising the silicon content degrades workability with respect to manufacturing processes and products. A number of attempts have been made to reduce eddy current loss by decreasing the thickness of the steel sheet, but in addition to the inherent difficulty of achieving the secondary recrystallization needed to obtain a Goss orientation there are a number of other problems involved, with respect to the manufacture of transformers and the like, and as for the same core loss thicker sheet is industrially preferable to thinner sheet, there is also a limit to how much sheet thickness can be reduced.

JP-B-51-12451 and JP-B-53-28375 describe methods for improving the core loss characteristics that a tension coating imparts to steel sheet, but the tensioning effect of these depends on the product orientation, which is to say, the magnetic flux density, and as described in pages 2981 to 2984 of the Journal of Applied Physics, Vol. 41 No. 7 (June 1970), the higher the magnetic flux density B₈ the greater the tensioning effect becomes. Thus, with commercial high magnetic flux density electrical steel sheet with a B₈ of around 1.92 tesla, there is a limit to how much the core loss characteristics can be improved. Techniques for lowering core loss by artificially fining domain size have been described by JP-B-58-5968 and JP-B-58-26405, but in these methods the core loss reduction effect depends on the magnetic flux density and is limited with respect to the degree of magnetic flux density in current commercial products.

Among the quickest ways to reduce core loss is by fining of secondary recrystallization grains, which was proposed by one of the present inventors in JP-B-57-9419. However, the fact that it is difficult to obtain high magnetic flux density when the size of secondary recrystallization grains is fined limits the use of secondary recrystallization fining as a means of reducing core loss. As the remaining means of reducing core loss, in JP-B-58-50295 the present applicants proposed a method of raising the magnetic flux density B₈ from the current level of around 1.92 tesla to a more ideal 2.03 tesla (the saturation magnetic flux density of 3% Si-Fe steel). For the first time this method stably provided a product with a very high magnetic flux density B₈ that far exceeded 1.92 tesla. However, the fact that the method involves the application of a temperature gradient during secondary recrystallization and that application of the method to a coil form with mill sizes is accompanied by a large loss of thermal energy as one end is heated as the other end is being cooled, are major problems with respect to commercial implementation.

The object of the present invention is to provide a grain-oriented electrical steel sheet and material having very high magnetic flux density and a method of manufacturing same, in place of the above described core loss reduction means.

As a result of careful, assiduous research into grain-oriented electrical steel sheet having very high magnetic flux density, the present inventors succeeded in stably obtaining a product having a very high magnetic flux density higher than the conventional 1.92 tesla, and upon analyzing the product discovered the first commercial means for obtaining very high magnetic flux density within the limits of the secondary recrystallization grain shape and the slope between ideal Goss orientation. That is, it was found that is was necessary for no fewer than 80 percent of grain diameters in the secondary recrystallization matrix to be 50 to 5 mm in the direction perpendicular to the cold rolling direction and 100 to 10 mm in the direction of the cold rolling and for no fewer than 50 percent of grain in the secondary recrystallization matrix to have an average grain diameter not greater than 5 mm, including fined secondary recrystallization grains, and that it was necessary for the crystalline orientation of secondary recrystallization grains and fined secondary recrystallization grains to be within 5 degrees and 10 degrees respectively of the ideal Goss around the TD axis and the ND axis, and that this needs to be the case with respect to no fewer than 90 percent of the grains.

With respect to the manufacture of high magnetic flux density grain-oriented steel sheet in which AlN is used as an inhibitor, it was confirmed that it could be obtained by adding bismuth or a bismuth-containing substance to the molten steel to achieve a ladle analysis content value of Bi = 0.0005 to 0.05 weight percent (hereinafter referred to simply as "percent"). While any of the various methods of manufacturing very high magnetic flux density grain-oriented electrical steel sheet that have been proposed may be followed, the following manufacturing method is also possible. Grain-oriented steel sheet less than 0.23 mm thick having a very high magnetic flux density may be manufactured by omitting preliminary cold rolling for the 50 percent or lower cold rolling reduction ratio considered desirable, and by using a full one-stage heavy reduction cold rolling method. It also became clear that, concerning the preferred industrial technique of using interpass aging treatment between cold rolling passes, that is to say, the reverse cold rolling method, with the composition system of the present invention the steel could be produced with tandem cold rolling without the aging treatment. Moreover, it was also found that in the case of the continuous high temperature annealing used prior to the final cold rolling, grain-oriented electrical steel sheet having very high magnetic flux density could be obtained using annealing at a lower temperature, and that with respect to the cooling following continuous high temperature annealing, a slower cooling rate could be used.

The invention will be described in detail in connection with the drawings, in which
Figure 1 shows the relationship between core loss W_{17/50} and magnetic flux density B₈ in 0.30-mm-thick grain-oriented electrical steel sheet containing 3 percent silicon that has been subjected to magnetic domain control by laser irradiation;
Figure 2 shows the relationship between magnetic flux density and grain diameter in the cold rolling direction in 0.30-mm-thick grain-oriented electrical steel sheet containing 3.25 percent silicon;
Figure 3 shows the relationship between magnetic flux density and grain diameter in the direction perpendicular to the cold rolling direction in 0.30-mm-thick grain-oriented electrical steel sheet containing 3.25 percent silicon;
Figure 4 shows, by content ratio of fine secondary recrystallization grains, the relationship between core loss W_{17/50} and magnetic flux density B₈ in 0.30-mm-thick grain-oriented electrical steel sheet containing 3 percent silicon.

The inventors carried out various studies on the conditions needed to provide a product with very high magnetic flux density, and by controlling the secondary recrystallization matrix grains and the fine secondary recrystallization grains in the secondary recrystallization matrix grains in grain-oriented electrical steel sheet containing 2.5 to 4.0 percent silicon, succeeded in developing grain-oriented electrical steel sheet having very high magnetic flux density and excellent core loss reduction effect.

Details of the invention will now be described, starting with details of composition conditions. By affecting the specific resistance of electrical steel sheet, the silicon content has a considerable influence on core loss properties. Therefore, a silicon content of less than 2.5 percent is undesirable as the specific resistance of the steel is thereby reduced, increasing the eddy current loss. On the other hand, a content that exceeds 4.0 percent is undesirable as it degrades workability, making it difficult to produce and process the steel.

The reasons for the limitations on the magnetic flux density will now be explained. Figure 1 shows the relationship between core loss and magnetic flux density B₈ in 3 percent silicon grain-oriented electrical steel sheet 0.30 mm thick from which the surface glass film has been removed by pickling, on which the measurement has been performed at a tension of 1.5 kg/mm₂ after laser beam irradiation at a 5 mm pitch perpendicular to the direction of cold rolling. As a W_{17/50} core loss falls below 1.0 W/kg, which is considered good even for a 0.30 mm product, with a flux density of 1.92 tesla or above, and a W_{17/50} core loss falls below 0.90 W/kg, which is considered particularly good, with a flux density of 1.95 tesla or above, in the present invention the magnetic flux density B₈ has been limited to not lower than 1.92 tesla.

Secondary recrystallization grain diameter, which is a main focus of the invention, will now be explained. As mentioned above, decreasing secondary recrystallization grain diameter usually tends to reduce the magnetic flux density, but in the case of this invention, the results shown in Figures 2 and 3 were obtained by the inventors after a study of the relationship between magnetic flux density and grain diameter in grain-oriented electrical steel sheet produced by various methods. The grain diameters were averaged with respect to the maximum lengths of grains of not less than 5 mm in diameter (excluding fine grains of less than 5 mm in the direction of the cold rolling) accounting for not less than 80 percent of the area of the secondary recrystallization grain matrix.

Figure 2 shows the relationship between grain diameter in the direction of the cold rolling and magnetic flux density. A magnetic flux density of 1.92 tesla or above is obtained stably in the case of grain diameters of not less than 10 mm in the secondary recrystallization grain matrix, and the attainment of 1.95 tesla is limited to grain diameters of not less than 10 mm.

Similarly, from Figure 3 it can be seen that a magnetic flux density of 1.92 tesla or above is obtained stably, or even an excellent 1.95 tesla or above is obtained, in the case of grain diameters of not less than 5 mm in the direction perpendicular to the cold rolling direction, and said excellent magnetic flux density of 1.95 tesla or above is virtually assured in the case of grain diameters of not less than 10 mm.

Next, with respect to the ratio of large grains in the secondary recrystallization grain matrix that are not smaller than the size limit, as shown by the above figures and explanation, secondary recrystallization grains less than 10 mm in diameter in the direction of the cold rolling and less than 5 mm in the direction perpendicular to the direction of cold rolling have a low magnetic flux density, and a ratio thereof that exceeds 20 percent will affect the magnetic flux density of the overall product and make it impossible to obtain a product having a magnetic flux density of 1.92 tesla or above, or a very high magnetic flux density of 1.95 tesla or above.

The state of fine secondary recrystallization in the matrix grains will now be explained. Figure 4 shows the relationship between core loss and magnetic flux density in grain-oriented electrical steel sheet product (with a tension coating) 0.30 mm thick containing 3 percent silicon. A rough correspondence can be seen between magnetic flux density and core loss, but unlike in the case of the laser-beam irradiated material of Figure 1, there is considerable variation in core loss values for the same magnetic flux density. The best core loss values were on a par with those of materials subjected to laser beam irradiation. As a result of detailed studies carried out by the inventors with respect to products having these good core loss values, it was found that, as classified in the figures, when the matrix secondary recrystallization grains include not fewer than 50 percent fine secondary recrystallization grains having a diameter not exceeding 5 mm, a product was obtained which at a flux density of 1.92 tesla or above had a W_{17/50} core loss of less than 1.0 W/kg, or at a flux density of 1.95 tesla or above had a W_{17/50} core loss of 0.95 W/kg.

While the mechanism of this core loss reduction is not clear, in the very high magnetic flux density grain-oriented electrical steel sheet at which the invention is directed, the inventors confirmed that when fine secondary recrystallization grains are not included, magnetic domain walls continue to pass through the crystal grains and thereby become coarser, whereas when fine secondary recrystallization grains are included, new magnetic domains are generated from the fine crystals, giving rise to a domain fining effect.

The crystal orientation distribution will now be explained. That a relationship exists between the magnetic flux density of a grain-oriented electrical steel sheet and the orientation of its secondary recrystallization grains is well known. Up to now, however, the literature has been silent on the orientation distribution when, as in the present invention, the sheet includes both coarse matrix secondary recrystallization grains and fine secondary recrystallization grains within the matrix grains. In particular, no teaching whatsoever has been published regarding the grain orientation distribution of grain-oriented electrical steel sheet which, like that of the present invention, exhibits a flux density of not less than 1.92 tesla and even up to the extremely high level of 1.95 tesla or higher.

The inventors measured the fine orientation distribution features of the very high magnetic flux density grain-oriented electrical steel sheet according to the invention and, as a result, obtained the following new knowledge. Specifically, they learned that for a very high magnetic flux density grain-oriented electrical steel sheet to exhibit a flux density B₈ of not less than 1.92 tesla, even of 1.95 tesla or higher, it is necessary that among the matrix secondary recrystallization grains not fewer than 90 percent be accounted for by grains whose {110} [001] axes are inclined relative to the rolled surface less than 5 degrees around either the TD axis or the ND axis, and that not fewer than 90 percent be accounted for by fine secondary recrystallization grains whose {110} [001] axes are inclined relative to the rolled surface less than 10 degrees around either the TD axis or the ND axis. Outside these ranges it is difficult to achieve the object of the invention, namely, to obtain a very high magnetic flux density grain-oriented electrical steel sheet exhibiting a flux density B₈ of not less than 1.92 tesla and even up to 1.95 tesla or higher.

Further explanation will now be given regarding the maximum diameter of the secondary recrystallization matrix grains referred to in the Summary of the Invention. The limitation of the grain diameter in the direction perpendicular to the cold rolling direction to not more than 50 mm is not required from the point of the magnetic properties and was set only because larger grains are seldom obtained in actual products. On the other hand, the grain diameter in the cold rolling direction has a bearing on the aforesaid orientation distribution. If the secondary recrystallization annealing is conducted in the flat state with respect to cut sheet segments, the limitation to not more than 100 mm set by the invention is not required as far as the relationship with grain orientation is concerned. In actual industrial production, however, the secondary recrystallization annealing is ordinarily conducted with respect to coiled sheet. In this case, if the diameter of the secondary recrystallization grains is long in the longitudinal direction of the coil, i.e., the cold rolling direction, the inclination of their {110} [001] axes relative to the rolled surface becomes large around the TD axis at the rear edges of the grains and may come to exceed the 5 degrees limit mentioned above. Because of this, the invention limits the length of the secondary recrystallization grains in the cold rolling direction to not more than 100 mm.

An explanation of the material constituents used for producing the very high magnetic flux density grain-oriented electrical steel sheet according to the invention will now be given, followed by an explanation of the production process. The very high magnetic flux density grain-oriented electrical steel sheet is produced from the same materials as used in the production of an ordinary high flux density grain-oriented electrical steel sheet using AlN as the main inhibitor, except that it further contains 0.0005 to 0.05 percent bismuth by weight. A high magnetic flux density grain-oriented electrical steel sheet using AlN as its main inhibitor is typically produced by a high temperature slab heating method in which the slab is heated to a high temperature of not lower than 1280°C at the time of hot rolling (as in the method of JP-B-46-23820) or by a low temperature slab heating method in which the slab is heated to a temperature that does not exceed 1270°C (as in the method of JP-A-59-56522). Either of these methods can be used for obtaining a very high magnetic flux density grain-oriented electrical steel sheet by addition of a small amount of bismuth in accordance with this invention. At a bismuth content of less than 0.0005 percent the improvement in flux density is slight, while at a content of more than 0.05 percent the effect of increasing flux density saturates, making addition of more than this amount uneconomical. Since a higher bismuth content also causes edge cracking during hot rolling, its upper limit is set at 0.05 percent. From the viewpoint of flux density improvement effect and negative economic effect (the cost increase and reduced yield from edge cracking resulting from bismuth addition), it is preferable for the bismuth content to be 0.0005 to 0.01 percent.

It is not altogether clear why bismuth affects secondary recrystallization, greatly increases flux density and changes the shape of the secondary recrystallization grains. However, an in-depth study conducted by the inventors has so far clarified the following points. First, there is the inhibitor effect of bismuth itself. Since bismuth has substantially no solid solubility in steel, it is already finely dispersed and exhibits inhibitor effect at the time of solidification. Since it is also unlikely to produce Ostwald growth in the temperature range of the secondary recrystallization, it retains its inhibitor effect up to high temperatures. Second, it also appears to affect the precipitation of AlN and MnS in such a manner as to enhance the fine distribution of these conventional inhibitors. Third, it was found that it changes the form of the oxides on the sheet surface during decarburization annealing, in this way strengthening the shielding effect with respect to the atmosphere during the secondary recrystallization annealing and thus changing the inhibitor effect through suppression of nitriding and denitriding.

Addition of bismuth during production of a grain-oriented electrical steel sheet material is taught by JP-A-50-72817, JP-A-51-78733 and JP-A-53-39922. However, these patents describe grain-oriented electrical steel sheets that fundamentally do not contain aluminum and in their specifications explain that bismuth is added in lieu of Sb, an intergranular segregation element. Therefore, differently from in the present invention, bismuth has to be added at not less than 0.01 to 0.02 percent. JP-A-51-107499 and JP-A-63-100127 also teach bismuth addition. Although these patents are similar to the present invention in the point of using AlN as the main inhibitor, like the aforementioned three patents they also define Sb as a substitute intergranular segregation element and require a bismuth content of not less than 0.01 to 0.02 percent. The present invention is thus totally different from these prior art references in technical idea and constitution.

An explanation will now be given with regard to the other material constituents.

C: In the high-temperature slab heating method, a carbon content of less than 0.03 percent is undesirable because it leads to abnormal grain growth during slab heating prior to hot rolling and results in a type of defective secondary recrystallization known as streaks. In the low-temperature slab heating method, a carbon content of less than 0.03 percent is undesirable because secondary recrystallization becomes unstable, and when it does occur, results in very poor magnetic flux density. On the other hand, a carbon content of more than 0.15 percent is undesirable from the industrial viewpoint because the decarburization becomes insufficient at a normal decarburization annealing time period, thus giving rise to magnetic aging in the product.

Si: A silicon content of less than 2.5 percent is undesirable because it increases the product eddy current loss, while a silicon content of greater than 4.0 percent is undesirable because it makes cold rolling difficult at normal temperature.

Mn: In the high-temperature slab heating method, an manganese content of 0.02 to 0.30 percent is necessary for precipitating MnS as an auxiliary inhibitor to AlN. A content below the lower limit is undesirable because the amount of inhibitor becomes insufficient. A content above the upper limit is undesirable because MnS remains undissolved during slab heating and forms coarse precipitates after hot rolling, which weakens the inhibitor effect and causes unstable secondary recrystallization. In the low-temperature slab heating method, a manganese content of 0.10 to 0.80 percent is necessary for obtaining a high magnetic flux density.

S: In the high-temperature slab heating method, a sulfur content of 0.005 to 0.040 percent is necessary for securing MnS as an auxiliary inhibitor. In the low-temperature slab heating method, a sulfur content of less than 0.010 percent is required for preventing partially defective secondary recrystallization owing to sulfur segregation.

Acid soluble Al: Acid soluble aluminum serves as a main inhibitor forming element in the production of a high magnetic flux density grain-oriented electrical steel sheet. In this point, it is also an important constituent in the present invention. An acid soluble aluminum content of less than 0.010 percent is undesirable because the amount of precipitated AlN becomes insufficient and lowers the inhibitor strength. On the other hand, at a content of more than 0.065 percent the AlN precipitates become coarse, and this also lowers the inhibitor strength.

N: Like acid soluble aluminum, nitrogen is a main inhibitor forming element. A content outside the range of 0.0030 to 0.0150 percent disrupts the optimum inhibitor state and, as such, is undesirable.

Sn: Tin is an element effective for stabilizing the secondary recrystallization of thin products. It is therefore required to be present at a content of not less than 0.05 percent. Its upper limit is set at 0.05 percent because its effect saturates above this level and addition of a greater amount only increases cost.

Cu: Copper is an element effective for improving the glass film produced by added tin. A content of less than 0.01 percent produces little effect, while a content in excess of 0.10 percent lowers the magnetic flux density of the product.

The production process conditions will now be explained. One feature of the present invention is the requirement that, in terms of bismuth, the bismuth addition to the molten steel be made at 100 to 5000 g per ton of molten steel. The source of the bismuth is not particularly limited and may be either metallic bismuth or a substance containing bismuth.

The molten steel whose composition has been adjusted in the foregoing manner is cast in the ordinary manner. The casting method is not particularly specified. The cast steel is then hot rolled into a hot-rolled coil. The slab heating temperature at the time of hot rolling preferably not less than 1280°C in the case of the high-temperature slab heating production method and not more than 1270°C in the case of the low-temperature slab heating method. The hot-rolled sheet is then subjected to a single stage cold rolling or several stages of cold rolling with interpass annealing to obtain a sheet of final thickness. Since the object is to obtain a high magnetic flux density grain-oriented electrical steel sheet, the final cold rolling reduction ratio (in the case of a single stage cold rolling, the reduction rate therefore) is preferably 65 to 95 percent. In this invention, it is possible to omit the not more than 50 percent reduction ratio that has been considered preferable in the production of a product with a thickness of not more than 0.23 mm (JP-A-59-126722) and to produce a thin product with a thickness of not more than 0.23 mm using the full single-stage one-time heavy reduction cold rolling method. This has not been possible heretofore because use of the full one-time heavy reduction cold rolling method to obtain a thin product with a thickness of not more than 0.23 mm causes a marked decrease in the number of Goss nuclei, so that with the inhibitors of the conventional composition the chance of secondary recrystallization is reduced, resulting in a product with defective secondary recrystallization grains. In this invention, however, the inhibitor strengthening effect obtained by addition of bismuth as explained earlier maintains the inhibitor effect up to high temperatures, making it possible to selectively grow Goss nuclei at the stage where the intergranular movement accelerates in the high-temperature region. This is thought to enable secondary recrystallization to proceed. Although the cold rolling with interpass aging described in JP-B-54-13846 is generally conducted at the time of cold rolling, with the composition of the present invention a product with excellent magnetic flux density can be obtained using the tandem cold rolling method without conducting interpass aging treatment. There is therefore no need to rely on this prior art.

Prior to final cold rolling, the sheet is subjected to the high-temperature annealing JP-B-46-23820 and then quenched. The composition of the present invention makes it possible to extend the range of the high-temperature annealing conditions. One condition that can be broadened is the annealing temperature. High-temperature annealing is ordinarily conducted at a temperature of 950 to 1200°C, preferably 1050 to 1200°C, and more preferably not less than 1100°C. With the composition of the present invention, however, it is possible to obtain a product with excellent magnetic flux density even when annealing is conducted within the temperature range of 850 to 1100°C. This is an advantage from the industrial viewpoint because it not only enables an energy saving proportional to the reduction in annealing temperature but also mitigates high-temperature annealing induced brittleness. It is also possible to broaden the quenching conditions. JP-B-46-23820 calls for conducting the quenching following high-temperature annealing at a cooling rate which lowers the temperature from 950°C to 400°C in 2 to 200 seconds. According to Figure 4 of this prior art reference, higher cooling rates are preferable for obtaining a product with high magnetic flux density. For example, this reference states that for obtaining a magnetic flux density of 1.92 tesla using an annealing temperature of 1150°C it is necessary for the cooling from 950°C to 400°C to be conducted in less than 20 seconds. With the composition of the present invention, however, the cooling condition can be extended toward the gradual cooling side. Specifically, a product exhibiting excellent magnetic flux density can be obtained even with gradual cooling in which the temperature is lowered from 950°C to 400°C in 30 seconds or more. In actual industrial scale production, milder cooling conditions make it easier to achieve uniform cooling and to mitigate sheet brittleness by softening the quenched structure. This relaxation of cooling conditions therefore has high industrial significance and can be expected to be vigorously pursued in conjunction with the improvement of core loss property through increased silicon content.

The sheet cold rolled to final product thickness is annealed and then subjected to decarburization annealing in the usual manner. Although the decarburization annealing method is not particularly specified, it is preferably conducted for 30 seconds to 30 minutes at 700 to 900°C in a mixed gas atmosphere consisting of wet hydrogen or hydrogen and nitrogen.

For preventing sticking during secondary recrystallization annealing and making a glass film, the surface of the decarburization annealed sheet is coated with an annealing separator of ordinary composition in the ordinary manner. The secondary recrystallization annealing is conducted for not less than 5 hours at a temperature of not less 1000°C in an atmosphere of hydrogen or nitrogen or a mixture of both.

After excess annealing separator has been removed, the sheet is subjected to continuous annealing to flatten a coil set. An insulating coating is applied and baked on at the same time. If necessary, magnetic domain fining treatment is conducted by irradiation with a laser beam or the like. The invention does not particularly specify the magnetic domain fining treatment method.

### Example 1

An electrical steel sheet slab comprising 0.06 to 0.09 percent carbon, 3.0 to 3.35 percent silicon, 0.08 percent manganese, 0.025 percent sulfur, 0.020 to 0.035 percent acid soluble aluminum, 0.008 percent nitrogen, 0 to 0.15 percent tin, 0 to 0.05 percent copper and 0.0005 to 0.05 percent bismuth and the balance of iron and unavoidable impurities, was heated to 1320°C and hot rolled to a sheet thickness of 2.3 mm. The hot rolled sheets were then cold rolled to obtain product sheets 0.30 mm and 0.23 mm thick, and between cold rollings some of these sheets were subjected to aging treatment 5 times at 200°C. Prior to final cold rolling high temperature annealing was applied at 1120°C for 2 minutes. The sheets were then subjected to decarburization annealing at 850°C, coated with an annealing separator in which the main constituent was MgO and then subjected to secondary recrystallization annealing at 1200°C. After removing the remaining annealing separator, pieces measuring 60 mm by 300 mm were cut as specimens to measure magnetic properties, and the specimens were annealed at 850°C to remove internal stresses. Next, an insulating coating was applied to the specimens and baked. The magnetic properties of some of the specimens were measured after the specimens were subjected to laser beam irradiation at 5 mm intervals. After then being pickled with strong acid, specimen grain diameter and the like were measured. The results are listed in Table 1.

Specimens 2 and 3 containing bismuth have a magnetic flux density exceeding 1.95 tesla and a ratio of large grains in the secondary recrystallization grain matrix exceeding 80 percent, and a core loss, following laser-beam irradiation, that is far lower than 0.90 W/kg, which for an 0.30 mm thick product can be described as excellent characteristics that surpass the limits of prior art products. Specimens 4 and 5 containing bismuth have a magnetic flux density exceeding 1.95 tesla, a ratio of large grains in the secondary recrystallization grain matrix exceeding 80 percent, and the matrix large grains also include are more than 50 percent fine secondary recrystallization grains, so that even without laser-beam treatment they exhibit core loss values not exceeding 0.95 W/kg, which can be described as particularly excellent characteristics for an 0.30 mm thick product. Specimens 9, 10 and 11 are 0.23 mm thick products and like 0.30 mm thick products are within the scope of the present invention, and as laser-beam irradiated products exhibit particularly good characteristics.

### Example 2

Specimens were prepared from 0.30 mm thick sheet produced by the same as Example 1, and the magnetic properties of the specimens were measured. Next, after pickling with strong acid, in each specimen the orientation of 20 crystal grains was measured, using the Laue method. The results are listed in Table 2.

As shown by Table 2, in specimens having a magnetic flux density of 1.95 tesla or higher, matrix grains having an angle of rotation from the ideal Goss, i.e., from the {110} [001] orientation, not exceeding 5 degrees, or not exceeding 10 degrees with respect to fine grains, accounted for not less than 90 percent in terms of area.

**TABLE 2**

| Magnetic flux density B⁸ (T) | Crystal Grain Orientation | | | |
|---|---|---|---|---|
| | Areal percentage of matrix large grains not exceeding 5 degrees | | Areal percentage of fine grains not exceeding 10 degrees | |
| | Around TD axis | Around ND axis | Around TD axis | Around ND axis |
| 1.903 | 85 | 70 | 80 | 60 |
| 1.935 | 90 | 90 | 90 | 70 |
| 1.983 | 100 | 95 | 95 | 95 |
| 2.005 | 100 | 100 | 100 | 95 |
| Note: Crystal orientation is indicated in terms of angle of rotation from ideal Goss orientation in the direction of cold rolling surface direction. | | | | |

### Example 3

0.0005 to 0.05 percent bismuth was added to steel containing 0.08 percent carbon, 3.05 percent silicon, 0.08 percent manganese, 0.025 percent sulfur, 0.025 percent acid soluble aluminum and 0.009 percent nitrogen. The slab was heated to 1320°C and hot rolled to a sheet thickness of 2.3 mm. The hot rolled sheets were then annealed at 1100°C, and after being pickled were subjected to aging treatment 5 times at 250°C between cold rolling passes, whereby the sheets were cold rolled to a sheet thickness of 0.30 mm. The sheets were then subjected to decarburization annealing at 850°C, coated with an annealing separator in which the main constituent was MgO and then subjected to secondary recrystallization finish annealing at 1200°C. Table 3 shows the relationship between bismuth content and magnetic flux density in the products thus obtained.

**TABLE 3**

| Bi content (%) | B₈ (T) |
|---|---|
| None added | 1.912 |
| 0.0005 | 1.971 |
| 0.002 | 2.003 |
| 0.010 | 2.008 |
| 0.050 | 1.978 |

From Table 3 it can be seen that, by adding bismuth, an excellent product was obtained having a magnetic flux density B₈ not lower than 1.95 tesla, which could not be obtained with the methods of the prior art.

### Example 4

0.009 percent bismuth was added to steel containing 0.09 percent carbon, 3.3 percent silicon, 0.07 percent manganese, 0.025 percent sulfur, 0.026 percent acid soluble aluminum, 0.009 percent nitrogen, 0.15 percent tin and 0 to 0.07 percent copper. The subsequent steps were the same as those of Example 3, except that the sheet was cold rolled to a thickness of 0.23 mm. The characteristics of the products thus obtained are listed in Table 4.

**TABLE 4**

| Bi content (%) | Cu content (%) | B₈ (T) |
|---|---|---|
| 0.009 | None added | 1.993 |
| 0.009 | 0.07 | 2.005 |

As is clear from Table 4, a product with excellent high magnetic flux density can be obtained by the addition of bismuth even to steel to which tin or tin and copper has been added.

### Example 5

The products obtained in Example 4 were subjected to magnetic domain fining treatment using laser-beam irradiation at a pitch of 5 mm. The results are listed in Table 5.

**TABLE 5**

| Bi content (%) | Cu content (%) | B₈ (T) | W_{17/50} (W/kg) |
|---|---|---|---|
| 0.009 | None added | 2.000 | 0.62 |
| 0.009 | 0.07 | 2.013 | 0.60 |

As is clear from Table 5, the specimens of this Example have a very high magnetic flux density and after grain fining attain an excellent core loss of 0.6 W/kg.

### Example 6

0.008 percent bismuth was added to steel containing 0.06 percent carbon, 3.2 percent silicon, 0.13 percent manganese, 0.007 percent sulfur, 0.028 percent acid soluble aluminum, 0.008 percent nitrogen and 0 to 0.12 percent tin. The slab was heated to 1150°C and hot rolled to a sheet thickness of 1.8 mm. The hot rolled sheets were then annealed at 1100°C, and after being pickled were subjected to aging treatment 5 times at 180°C between cold rolling passes, whereby the sheets were cold rolled to a thickness of 0.23 mm, subjected to decarburization annealing at 830°C and then subjected to nitriding treatment for 30 seconds at 750°C in an atmosphere containing ammonium. The steel sheets were then coated with an annealing separator in which the main constituent was MgO and subjected to finish annealing at 1200°C. The characteristics of the products thus obtained are listed in Table 6.

**TABLE 6**

| Bi content (%) | Sn content (%) | B₈ (T) |
|---|---|---|
| 0.008 | None added | 1.988 |
| 0.008 | 0.12 | 1.992 |

As is clear from Table 6, a product with very high magnetic flux density can be obtained by the addition of bismuth even to steel thus produced the low-temperature slab heating method.

### Example 7

100 to 5000 g(/melt T) metallic bismuth was added to a steel melt containing 0.08 percent carbon, 2.98 percent silicon, 0.08 percent manganese, 0.023 percent sulfur, 0.025 percent acid soluble aluminum and 0.008 percent nitrogen. The same steps as those of Example 3 were used, and the magnetic characteristics of the products were measured. The results are listed in Table 7.

**TABLE 7**

| Added Bi (g/molten steel T) | B₈ (T) |
|---|---|
| None added | 1.919 |
| 100 | 1.958 |
| 500 | 1.998 |
| 1000 | 2.002 |
| 5000 | 1.973 |

From Table 7 it can be seen that, by adding metallic bismuth, an excellent product was obtained having a magnetic flux density B₈ not lower than 1.95 tesla, which could not be obtained with the methods of the prior art.

### Example 8

No bismuth or 0.010 percent bismuth was added to steel containing 0.08 percent carbon, 3.05 percent silicon, 0.08 percent manganese, 0.025 percent sulfur, 0.026 percent acid soluble aluminum and 0.008 percent nitrogen. The slabs were heated to 1320°C and rolled to a sheet thickness of 2.3 mm. The hot rolled sheets were then annealed at 1100°C and, after being pickled, were either subjected to aging treatment 5 times at 250°C between cold rolling passes or not subjected to aging treatment, whereby cold rolled sheets 0.30 mm thick were obtained using two sets of conditions. The sheets were then subjected to decarburization annealing at 850°C, coated with an annealing separator in which the main constituent was MgO and then subjected to secondary recrystallization finish annealing at 1200°C. The results of the magnetic measurements are listed in Table 8.

**TABLE 8**

| Bi content (%) | Interpass aging applied? Yes No | B₈ (T) |
|---|---|---|
| None added | Yes | 1.917 |
| | No | 1.882 |
| 0.010 | Yes | 1.997 |
| | No | 2.001 |

It can be seen from Table 8 that products with very high magnetic flux density could be obtained through the addition of bismuth, and that even when no interpass aging was used, unlike when no bismuth was added there was either no degradation in the magnetic flux density or there was a slight improvement. This is the direct opposite to what is anticipated when the prior art technologies are used.

### Example 9

No bismuth or 0.006 percent bismuth was added to steel containing 0.09 percent carbon, 3.2 percent silicon, 0.08 percent manganese, 0.026 percent sulfur, 0.026 percent acid soluble aluminum, 0.008 percent nitrogen, 0.15 percent tin and 0.07 percent copper. The slabs were heated to 1320°C and rolled to a sheet thickness of 2.3 mm. The hot rolled sheets were then annealed at 850°C to 1100°C and, after being pickled, were either subjected to aging treatment 5 times at 250°C between cold rolling passes or not subjected to aging treatment, whereby cold rolled sheets 0.30 mm thick were obtained. The sheets were then subjected to decarburization annealing at 850°C, coated with an annealing separator in which the main constituent was MgO and then subjected to secondary recrystallization finish annealing at 1200°C. Table 9 shows the relationship between bismuth content, hot-rolled sheet annealing temperature, the number of bending repetitions the annealed sheets were subjected to and the magnetic flux density B₈ of the product sheets.

**TABLE 9**

| Bi content (%) | Annealing temperature (°C) | No. of bendings | B₈ (T) |
|---|---|---|---|
| None added | 950 | >20 | 1.817 |
| | 1120 | 4 | 1.915 |
| 0.006 | 850 | >20 | 1.953 |
| | 1050 | 18 | 1.991 |
| 0.009 | 1150 | 2 | 1.968 |

It can be seen from Table 9 that by adding bismuth, products could be obtained having a very high magnetic flux density not achievable with the methods of the prior art, and that even with a hot-rolled sheet annealing temperature not exceeding 1100°C, unlike when no bismuth was added there was either no degradation in the magnetic flux density or there was a slight improvement. Such an effect cannot be anticipated from the prior art. Furthermore, while with an annealing temperature that does exceed 1100°C the number of bendings of the annealed sheet is less than the 5 that is used as a guide in the case of commercial sheet on a continuous line, with the steel of the present invention to which bismuth has been added, more than 5 bendings can be ensured with an annealing temperature not exceeding 1100°C.

### Example 10

No bismuth or 0.010 percent bismuth was added to steel containing 0.09 percent carbon, 3.3 percent silicon, 0.07 percent manganese, 0.025 percent sulfur, 0.027 percent acid soluble aluminum, 0.009 percent nitrogen and 0.15 percent tin. The hot rolled sheets were annealed at 1050°C and then cooled either by quenching in 100°C water, or by forced air-cooling, or by atmospheric cooling, and after being pickled the sheets were cold rolled to a thickness of 0.30 mm. The sheets were then subjected to decarburization annealing at 850°C, coated with an annealing separator in which the main constituent was MgO and then subjected to secondary recrystallization finish annealing at 1200°C. Table 10 shows the relationship between bismuth content, hot-rolled sheet annealing and cooling conditions, the number of bending repetitions the annealed sheets were subjected to and the magnetic flux density B₈ of the product sheets.

**TABLE 10**

| Bi content (%) | Cooling conditions | Cooling rate °C/s | No. of bendings | B₈ (T) |
|---|---|---|---|---|
| None added | Quenched in 100°C water | 30 | 8 | 1.919 |
| | Atmospheric cooling | 4 | >20 | 1.852 |
| 0.010 | Quenched in 100°C water | 30 | 2 | 1.968 |
| | Forced air-cooling | 13 | 18 | 1.982 |
| | Atmospheric cooling | 4 | >20 | 1.961 |

It can be seen from Table 10 that by adding bismuth, products could be obtained having a very high magnetic flux density not achievable with the methods of the prior art, and that even when the annealing is followed by gradual cooling in water no hotter than 100°C, unlike when no bismuth was added there was either no degradation in the magnetic flux density or there was a slight improvement. Such an effect cannot be anticipated from the prior art. Furthermore, while with a cooling rate of 30°C/s the number of bendings of the annealed sheet is less than the 5 that is used as a guide in the case of commercial sheet on a continuous line, with the steel of the present invention to which bismuth has been added, more than 5 bendings can be ensured with the gradual cooling conditions used.

## Claims

1. Very high magnetic flux density grain-oriented electrical steel sheet produced from a slab comprising, by weight, 0.03 to 0.15 percent carbon, 2.5 to 4.0 percent silicon, 0.02 to 0.30 percent manganese, 0.005 to 0.040 percent sulfur, 0.010 to 0.065 percent acid soluble aluminum, 0.0030 to 0.0150 percent nitrogen, 0.0005 to 0.05 percent bismuth, optionally 0.05 to 0.50 percent tin and/or 0.01 to 0.10 percent copper, and the balance of iron and unavoidable impurities, and having a very high magnetic flux density B₈ of not less than 1.92 tesla, in which by area not less than 80 percent is accounted for by matrix secondary recrystallization grains having a diameter not larger than 100 mm and not smaller than 10 mm in a direction of cold rolling and not larger than 50 mm and not smaller than 5 mm in a direction perpendicular to the cold rolling direction, and in which, moreover, of the grains in said matrix, not fewer than 50 percent are fine secondary recrystallization grains having an average diameter not larger than 5 mm, wherein bismuth and acid soluble aluminum are contained as inhibitor components.

2. The very high magnetic flux density grain-oriented electrical steel sheet according to claim 1, in which of the matrix secondary recrystallization grains not fewer than 90 percent are accounted for by grains whose {110} [001] axes are inclined relative to the rolled surface less than 5 degrees around either the TD axis or the ND axis, and not fewer than 90 percent are accounted for by fine secondary recrystallization grains whose {110} [001] axes are inclined relative to the rolled surface less than 10 degrees around either the TD axis or the ND axis.

3. Very high magnetic flux density grain-oriented electrical steel sheet produced from a slab comprising, by weight, 0.03 to 0.15 percent carbon, 2.5 to 4.0 percent silicon, 0.10 to 0.80 percent manganese, up to 0.010 percent sulfur, 0.010 to 0.065 percent acid soluble aluminum, 0.0030 to 0.0150 percent nitrogen, 0.0005 to 0.05 percent bismuth, optionally 0.05 to 0.50 percent tin and/or 0.01 to 0.10 percent copper, and the balance of iron and unavoidable impurities, and having a very high magnetic flux density B₈ of not less than 1.92 tesla, in which by area not less than 80 percent is accounted for by matrix secondary recrystallization grains having a diameter not larger than 100 mm and not smaller than 10 mm in a direction of cold rolling and not larger than 50 mm and not smaller than 5 mm in a direction perpendicular to the cold rolling direction, and in which, moreover, of the grains in said matrix, not fewer than 50 percent are fine secondary recrystallization grains having an average diameter not larger than 5 mm, wherein bismuth and acid soluble aluminum are contained as inhibitor components.

4. A method of manufacturing very high magnetic flux density grain-oriented electrical steel sheet according to any one of claims 1 to 3 comprising the steps of casting very high magnetic flux density grain-oriented electrical steel sheet material to form a steel slab, heating the slab, hot rolling the slab, if necessary carrying out high-temperature annealing prior to final cold rolling and cooling the steel, cold rolling the steel in a single stage or in two or more stages with an intermediate annealing therebetween including final cold rolling at a reduction ratio of 65 to 95 percent, decarburization annealing and application of annealing separator, and secondary recrystallization finish annealing, wherein bismuth or a compound containing bismuth in a bismuth equivalent amount of 100 to 5000 g/(ton of molten steel) is added to the molten steel, whereby bismuth and acid soluble aluminum result in as inhibitor components.

5. A method of manufacturing very high magnetic flux density grain-oriented electrical steel sheet according to claim 4, wherein the slab comprises, by weight, 0.02 to 0.30 percent manganese, 0.005 to 0.040 percent sulfur, and the slab is heated to at least 1,280 °C.

6. A method of manufacturing very high magnetic flux density grain-oriented electrical steel sheet according to claim 4, wherein the slab comprises, by weight, 0.10 to 0.80 percent manganese, up to 0.010 percent sulfur, the slab is heated to not more than 1,270 °C, and the decarburization annealing is followed by nitriding treatment.

7. A method of manufacturing very high magnetic flux density grain-oriented electrical steel sheet according to any one of claims 4 to 6, comprising obtaining a product thickness of 0.23 mm to 0.15 mm by a single stage heavy reduction cold rolling.

8. A method of manufacturing very high magnetic flux density grain-oriented electrical steel sheet according to any of claims 4 to 7, comprising tandem cold rolling.

9. A method of manufacturing very high magnetic flux density grain-oriented electrical steel sheet according to any of claims 4 to 8, comprising high-temperature annealing at 850°C to 1100°C for between 30 seconds and 30 minutes, prior to final cold rolling.

10. A method of manufacturing very high magnetic flux density grain-oriented electrical steel sheet according to any of claims 4 to 9, comprising following high-temperature annealing by cooling from no higher than 950°C down to 400°C at a rate that is slower than 30°C/s, prior to final cold rolling.

## Patentansprüche

1. Kornorientiertes Elektrostahlblech mit sehr hoher magnetischer Flußdichte, das aus einer Bramme mit den folgenden Bestandteilen in Gew.-% hergestellt ist: 0,03 bis 0,15% Kohlenstoff, 2,5 bis 4,0% Silizium, 0,02 bis 0,30% Mangan, 0,005 bis 0,040% Schwefel, 0,010 bis 0,065% säurelösliches Aluminium, 0,0030 bis 0,0150% Stickstoff, 0,0005 bis 0,05% Wismut, wahlweise 0,05 bis 0,50% Zinn und/oder 0,01 bis 0,10% Kupfer, wobei der Rest aus Eisen und unvermeidbaren Verunreinigungen besteht, und das eine sehr hohe magnetische Flußdichte B₈ von nicht weniger als 1,92 Tesla aufweist, wobei nicht weniger als 80% der Fläche von einer Matrix sekundär rekristallisierter Körner mit einem Durchmesser von nicht mehr als 100 mm und nicht weniger als 10 mm in Kaltwalzrichtung und von nicht mehr als 50 mm und nicht weniger als 5 mm senkrecht zur Kaltwalzrichtung eingenommen wird, und wobei außerdem von den Körnern in der Matrix nicht weniger als 50% feine sekundär rekristallisierte Körner mit einem mittleren Durchmesser von nicht mehr als 5 mm sind, wobei Wismut und säurelösliches Aluminium als Inhibitorkomponenten enthalten sind.

2. Kornorientiertes Elektrostahlblech mit sehr hoher magnetischer Flußdichte nach Anspruch 1, wobei von den sekundär rekristallisierten Körnern der Matrix nicht weniger als 90% Körner sind, deren {110}[001]-Achsen entweder um die TD-Achse oder um die ND-Achse um weniger als 5 Grad gegen die Walzoberfläche geneigt sind, und wobei nicht weniger als 90% feine sekundär rekristallisierte Körner sind, deren {110}[001]-Achsen entweder um die TD-Achse oder um die ND-Achse um weniger als 10 Grad gegen die Walzoberfläche geneigt sind.

3. Kornorientiertes Elektrostahlblech mit sehr hoher magnetischer Flußdichte, das aus einer Bramme mit den folgenden Bestandteilen in Gew.-% hergestellt ist: 0,03 bis 0,15% Kohlenstoff, 2,5 bis 4,0% Silizium, 0,10 bis 0,80% Mangan, bis zu 0,010% Schwefel, 0,010 bis 0,065% säurelösliches Aluminium, 0,0030 bis 0,0150% Stickstoff, 0,0005 bis 0,05% Wismut, wahlweise 0,05 bis 0,50% Zinn und/oder 0,01 bis 0,10% Kupfer, wobei der Rest aus Eisen und unvermeidbaren Verunreinigungen besteht, und das eine sehr hohe magnetische Flußdichte B₈ von nicht weniger als 1,92 Tesla aufweist, wobei nicht weniger als 80% der Fläche von einer Matrix sekundär rekristallisierter Körner mit einem Durchmesser von nicht mehr als 100 mm und nicht weniger als 10 mm in Kaltwalzrichtung und von nicht mehr als 50 mm und nicht weniger als 5 mm senkrecht zur Kaltwalzrichtung eingenommen wird, und wobei außerdem von den Körnern in der Matrix nicht weniger als 50% feine sekundär rekristallisierte Körner mit einem mittleren Durchmesser von nicht mehr als 5 mm sind, wobei Wismut und säurelösliches Aluminium als Inhibitorkomponenten enthalten sind.

4. Verfahren zur Herstellung von kornorientiertem Elektrostahlblech mit sehr hoher magnetischer Flußdichte nach einem der Ansprüche 1 bis 3, mit den folgenden Schritten: Gießen eines Materials für kornorientiertes Elektrostahlblech mit sehr hoher magnetischer Flußdichte zu einer Stahlbramme, Erwärmen der Bramme, Warmwalzen der Bramme, nötigenfalls Ausführen eines Hochtemperaturglühens vor dem Kaltfertigwalzen und Abkühlen des Stahls, einstufiges oder zwei- oder mehrstufiges Kaltwalzen des Stahls mit Zwischenglühen einschließlich des Kaltfertigwalzens mit einem Reduktionsgrad von 65 bis 95%, entkohlendes Glühen und Aufbringen eines Glühtrennmittels, und Fertigglühen zur sekundären Rekristallisation, wobei dem geschmolzenen Stahl Wismut oder eine wismuthaltige Verbindung in einem äquivalenten Wismutanteil von 100 bis 5000 g/(Tonne geschmolzener Stahl) zugesetzt wird, wodurch Wismut und säurelösliches Aluminium als Inhibitorkomponenten resultieren.

5. Verfahren zur Herstellung von kornorientiertem Elektrostahlblech mit sehr hoher magnetischer Flußdichte nach Anspruch 4, wobei die Bramme in Gew.-% 0,02 bis 0,30% Mangan und 0,005 bis 0,040% Schwefel aufweist und auf mindestens 1280°C erwärmt wird.

6. Verfahren zur Herstellung von kornorientiertem Elektrostahlblech mit sehr hoher magnetischer Flußdichte nach Anspruch 4, wobei die Bramme in Gew.-% 0,10 bis 0,80% Mangan und bis zu 0,010% Schwefel aufweist, wobei die Bramme auf nicht mehr als 1270°C erwärmt wird, und wobei sich an das entkohlende Glühen eine Nitrierbehandlung anschließt.

7. Verfahren zur Herstellung von kornorientiertem Elektrostahlblech mit sehr hoher magnetischer Flußdichte nach einem der Ansprüche 4 bis 6, wobei eine Produktdicke von 0,23 mm bis 0,15 mm durch einstufiges Kaltwalzen mit hohem Reduktionsgrad erzielt wird.

8. Verfahren zur Herstellung von kornorientiertem Elektrostahlblech mit sehr hoher magnetischer Flußdichte nach einem der Ansprüche 4 bis 7 mit Tandemkaltwalzen.

9. Verfahren zur Herstellung von kornorientiertem Elektrostahlblech mit sehr hoher magnetischer Flußdichte nach einem der Ansprüche 4 bis 8, das ein Hochtemperaturglühen bei 850°C bis 1100°C über 30 Sekunden bis 30 Minuten vor dem Kaltfertigwalzen aufweist.

10. Verfahren zur Herstellung von kornorientiertem Elektrostahlblech mit sehr hoher magnetischer Flußdichte nach einem der Ansprüche 4 bis 9, das anschließend an das Hochtemperaturglühen eine Abkühlung von höchstens 950°C auf 400°C mit einer Geschwindigkeit von weniger als 30°C/s vor dem Kaltfertigwalzen aufweist.

## Revendications

1. Tôle d'acier électrique à grains orientés à très haute densité de flux magnétique produite à partir d'une brame comprenant, en poids, de 0,03 à 0,15 pour cent de carbone, de 2,5 à 4,0 pour cent de silicium, de 0,02 à 0,30 pour cent de manganèse, de 0,005 à 0,040 pour cent de soufre, de 0,010 à 0,065 pour cent d'aluminium soluble dans un acide, de 0,0030 à 0,0150 pour cent d'azote, de 0,0005 à 0,05 pour cent de bismuth optionnellement de 0,05 à 0,50 pour cent d'étain et/ou de 0,01 à 0,10 pour cent de cuivre et le reste du fer et des impuretés inévitables, et ayant une très haute densité de flux magnétique B₈ non inférieure à 1,92 tesla dans laquelle, pas moins de 80 pour cent en superficie sont constitués de grains de recristallisation secondaire de matrice ayant un diamètre non supérieur à 100 mm et non inférieur à 10 mm dans une direction de laminage à froid et pas supérieur à 50 mm et pas inférieur à 5 mm dans une direction perpendiculaire à la direction de laminage à froid et dans laquelle en outre, parmi les grains dans ladite matrice, pas moins de 50 pour cent sont des grains de recristallisation secondaire fins ayant un diamètre moyen non supérieur à 5 mm, dans laquelle le bismuth et l'aluminium soluble dans un acide sont contenus en tant que composants inhibiteurs.

2. Tôle d'acier électrique à grains orientés à très haute densité de flux magnétique selon la revendication 1,
dans laquelle, parmi les grains de recristallisation secondaire de matrice, pas moins de 90 pour cent sont constitués de grains dont les axes (110) [001] sont inclinés, par rapport à la surface laminée, de moins de 5 degrés autour soit de l'axe TD, soit de l'axe ND, et pas moins de 90 pour cent sont constitués de grains de recristallisation secondaire fins dont les axes (110) [001] sont inclinés, par rapport à la surface laminée, de moins de 10 degrés autour soit de l'axe TD, soit de l'axe ND.

3. Tôle d'acier électrique à grains orientés à très haute densité de flux magnétique produite à partir d'une brame comprenant, en poids, de 0,03 à 0,15 pour cent de carbone, de 2,5 à 4,0 pour cent de silicium, de 0,10 à 0,80 pour cent de manganèse, jusqu'à 0,010 pour cent de soufre, de 0,010 à 0,065 pour cent d'aluminium soluble dans un acide, 0,0030 à 0,0150 pour cent d'azote, de 0,0005 à 0,05 pour cent de bismuth, optionnellement de 0,05 à 0,50 pour cent d'étain et/ou de 0,01 à 0,10 pour cent de cuivre et le reste du fer et des impuretés inévitables, et ayant une très haute densité de flux magnétique B₈ non inférieure à 1,92 tesla dans laquelle, pas moins de 80 pour cent en superficie sont constitués de grains de recristallisation secondaire de matrice ayant un diamètre non supérieur à 100 mm et non inférieur à 10 mm dans une direction de laminage à froid et pas supérieur à 50 mm et pas inférieur à 5 mm dans une direction perpendiculaire à la direction de laminage à froid et dans laquelle en outre, parmi les grains dans ladite matrice, pas moins de 50 pour cent sont des grains de recristallisation secondaire fins ayant un diamètre moyen non supérieur à 5 mm, dans laquelle le bismuth et l'aluminium soluble dans un acide sont contenus en tant que composants inhibiteurs.

4. Un procédé de fabrication d'une tôle d'acier électrique à grains orientés à très haute densité de flux magnétique selon l'une quelconque des revendications 1 à 3, comprenant les étapes de coulée d'un matériau de tôle d'acier électrique à grains orientés à très haute densité de flux magnétique pour former une brame d'acier, chauffage de la brame, laminage à chaud de la brame, si nécessaire exécution d'un recuit à haute température avant laminage à froid final et refroidissement de l'acier, laminage à froid de l'acier en une seule étape, ou en deux étapes ou plus avec un recuit intermédiaire entre elles incluant un laminage à froid final à un taux de réduction de 65 à 95 pour cent, recuit de décarburation et application d'un séparateur de recuit, et recuit de finition de recristallisation secondaire, dans lequel du bismuth ou un composé contenant du bismuth est ajouté à l'acier fondu en quantité équivalente de bismuth de 100 à 5000 g/tonne d'acier fondu, grâce à quoi le bismuth et l'aluminium soluble dans un acide résultent en des composants inhibiteurs.

5. Un procédé de fabrication d'une tôle d'acier électrique à grains orientés à très haute densité de flux magnétique selon la revendication 4,
dans laquelle la brame contient, en poids, de 0,02 à 0,30 pour cent de manganèse, de 0,005 à 0,040 pour cent de soufre et la brame est chauffée à au moins 1.280 °C.

6. Un procédé de fabrication d'une tôle d'acier électrique à grains orientés à très haute densité de flux magnétique selon la revendication 4,
dans laquelle la brame contient, en poids, de 0,10 à 0,80 pour cent de manganèse, jusqu'à 0,010 pour cent de soufre, la brame est chauffée à pas plus de 1.270 °C et le recuit de décarburation est suivi par un traitement de nitruration.

7. Un procédé de fabrication d'une tôle d'acier électrique à grains orientés à très haute densité magnétique selon l'une quelconque des revendications 4 à 6,
comprenant l'obtention d'une épaisseur de produit de 0,23 mm à 0,15 mm par un laminage à froid de réduction lourde en une étape.

8. Un procédé de fabrication d'une tôle d'acier électrique à grains orientés à très haute densité magnétique selon l'une quelconque des revendications 4 à 7,
comprenant un laminage à froid tandem.

9. Un procédé de fabrication d'une tôle d'acier électrique à grains orientés à très haute densité magnétique selon l'une quelconque des revendications 4 à 8,
comprenant un recuit à haute température à 850°C à 1100°C pendant, entre 30 secondes et 30 minutes, avant le laminage à froid final.

10. Un procédé de fabrication d'une tôle d'acier électrique à grains orientés à très haute densité magnétique selon l'une quelconque des revendications 4 à 9,
comprenant un recuit à haute température suivant par refroidissement de pas plus de 950°C à 400°C à une vitesse qui est inférieure à 30°C/s, avant le laminage à froid final.
